



US005202151A

**United States Patent [19]****Ushio et al.**

[11] **Patent Number:** **5,202,151**  
 [45] **Date of Patent:** **Apr. 13, 1993**

[54] **ELECTROLESS GOLD PLATING SOLUTION, METHOD OF PLATING WITH GOLD BY USING THE SAME, AND ELECTRONIC DEVICE PLATED WITH GOLD BY USING THE SAME**

[75] **Inventors:** **Jiro Ushio, Yokohama; Osamu Miyazawa, Yokosuka; Akira Tomizawa, Yokohama; Hitoshi Yokono, Ibaraki; Naoya Kanda; Naoko Matsuura, both of Yokohama; Setsuo Ando, Kawasaki; Hiroaki Okudaira, Yokohama, all of Japan**

[73] **Assignee:** **Hitachi, Ltd., Tokyo, Japan**

[21] **Appl. No.:** **532,656**

[22] **Filed:** **Jun. 4, 1990**

**Related U.S. Application Data**

[60] Division of Ser. No. 184,061, Apr. 20, 1988, Pat. No. 4,963,974, which is a continuation-in-part of Ser. No. 143,959, Jan. 14, 1988, Pat. No. 4,880,464, which is a continuation of Ser. No. 918,498, Oct. 14, 1986, abandoned.

**Foreign Application Priority Data**

Oct. 14, 1985 [JP] Japan ..... 60-226738  
 Apr. 18, 1986 [JP] Japan ..... 61-88269

[51] **Int. Cl. 5** ..... **C23C 26/00**

[52] **U.S. Cl.** ..... **427/98; 427/304;**

**427/305; 427/306; 427/443.1; 427/437**

[58] **Field of Search** ..... **427/98, 304, 305, 306,**  
**427/443.1, 437**

**References Cited****U.S. PATENT DOCUMENTS**

3,300,328 1/1967 Luce ..... 427/437  
 3,650,803 3/1972 Lin ..... 427/437  
 3,853,589 12/1974 Andrews ..... 427/304  
 4,009,297 2/1977 Redmond ..... 427/304

|           |         |           |           |
|-----------|---------|-----------|-----------|
| 4,154,877 | 5/1979  | Vratny    | 427/437   |
| 4,284,666 | 8/1981  | Feldstein | 427/304   |
| 4,474,838 | 10/1984 | Halecky   | 427/98    |
| 4,482,596 | 11/1984 | Gulla     | 427/443.1 |
| 4,657,632 | 4/1987  | Holtzman  | 427/437   |
| 4,711,835 | 12/1987 | Dufour    | 427/96    |
| 4,804,559 | 2/1989  | Ushio     | 427/98    |
| 4,880,464 | 11/1989 | Ushio     | 106/1.26  |
| 4,963,974 | 10/1990 | Ushio     | 174/250   |

**FOREIGN PATENT DOCUMENTS**

219788 4/1987 European Pat. Off. ..... 427/304  
 150762 4/1980 Fed. Rep. of Germany .

*Primary Examiner*—Shrive Beck

*Assistant Examiner*—Vi Duong Dang

*Attorney, Agent, or Firm*—Antonelli, Terry, Stout & Kraus

**[57] ABSTRACT**

The present invention relates to an electroless gold plating solution, a method of plating by using the same, and an electronic device plated with gold by using the same.

According to the present electroless gold plating solution, the plating solution components contain no cyanide ions, the amount of a reducing agent used is small, and gold plating can be carried out without causing the gold plating on conducting paths having a fine interval between them to short-circuit the conducting paths.

Therefore, according to the method of gold plating by using said electroless gold plating solution, a plating method that is safe in the plating work and in the treatment of its waste liquor can be accomplished. The method has a feature that the method can provide an electronic device on which parts can be mounted highly densely, and wherein the joint reliability to the parts is high.

**14 Claims, 9 Drawing Sheets**



FIG. 1



FIG. 2



FIG. 3



FIG. 4



FIG. 5



FIG. 6



FIG. 7



FIG. 8



FIG. 9



FIG. 10



FIG. 11



FIG. 12(a)



FIG. 12(b)



FIG. 13



FIG. 14



FIG. 15



FIG. 16



FIG. 17



FIG. 18



FIG. 19(a)



FIG. 19(b)



FIG. 20(a)



FIG. 20(b)



FIG. 21



FIG. 22



FIG. 23



FIG. 24



FIG. 25



FIG. 26



FIG. 27(a)



FIG. 27(b)



FIG. 27(c)



FIG. 27(d)



FIG. 27(e)



FIG. 27(f)



**ELECTROLESS GOLD PLATING SOLUTION,  
METHOD OF PLATING WITH GOLD BY USING  
THE SAME, AND ELECTRONIC DEVICE PLATED  
WITH GOLD BY USING THE SAME**

This application is a divisional application of application Ser. No. 07/184,061, filed Apr. 20, 1988, now U.S. Pat. No. 4,963,974 which is a continuation-in-part application of application Ser. No. 143,959, filed Jan. 14, 1988, now U.S. Pat. No. 4,880,464 which is a continuation application of application Ser. No. 918,498, filed Oct. 14, 1986, now abandoned.

**BACKGROUND OF THE INVENTION**

The present invention relates to an electroless gold plating solution, a method of plating with gold by using the same, and an electronic device plated by using the same.

As a prior electroless gold plating solution is known one containing, as major components, potassium dicyanoaurate (I), potassium cyanide, and a borane compound as disclosed in "Plating", Vol. 57 (1970), pages 914 to 920. According to the technique, a plating solution having a deposition rate of 1  $\mu\text{m}/\text{h}$  can be obtained. However, if the electroless gold plating solution is applied to circuit boards having surface conducting paths with the interval between the conducting paths small, gold is liable to deposit even on the insulator surface between the conducting paths. In addition, the electroless gold plating solution contains a large amount of cyanide ions, which causes safety problems in the plating operation and in the treatment of its waste solution.

As an electroless gold plating solution that contain no cyanide ions, one containing, as major components, tetrachloroaurate (III) and hydrazine is disclosed in U.S. Patent No. 3,300,328, and one containing, as major components, potassium tetrachloroaurate (III) and a borane compound is disclosed in Japanese Patent Publication No. 20353/1981. However, the electroless gold plating solutions disclosed in U.S. Pat. No. 3,300,328, and Japanese Patent Publication No. 20353/1981 have the problem that because the gold ion in the gold complex is trivalent a larger amount of a reducing agent is required in comparison with the case using potassium dicyanoaurate (I). Further, the electroless gold plating solution disclosed in U.S. Pat. No. 3,300,328 has such a problem that it is unstable to cause precipitation in the plating solution within about 2 hours, which does not allow the continuation of the plating.

Now the relationship between gold plating and electronic devices will be described. Electronic computers can be mentioned as a typical example where this relationship is most conspicuously noticed. As described in "Saiensu", Vol. 13 (1983), pages 13 to 25, in electronic computers, it is possible to decrease the delay of electric signals due to a circuit board by mounting semiconductor chips on the circuit board highly densely, and as a result the computing speed of the electronic computer can be improved. To increase the packing density of semiconductor chips, it is required to increase the density of the surface conducting paths of the circuit board. On the other hand, to join semiconductor chips by soldering, and to carry out engineering change such as wiring alteration by wire bonding, it is required that the top surface of the surface conducting paths of the circuit board is covered with metal layers made of gold. In

particular, the thickness of metal film at the surface conducting paths where wire bonding will be effected has to be 0.5  $\mu\text{m}$  or over to guarantee the joint reliability of the wire bonding. Consequently, to improve the packing density of semiconductor chips, namely, to realize a high-speed electronic computer, it is essential to provide a method of forming a gold film having a thickness of 0.5  $\mu\text{m}$  or over on conducting paths that are electroplating and are highly dense and complicated in shape.

Hitherto, electroplating has been used widely to form a gold film having a thickness of 0.5  $\mu\text{m}$  or over on a conductor by plating. However, if the above circuit board is plated with gold, then for electrically isolated conducting paths that are present in great numbers on the circuit board, conducting paths for continuity are to be formed between the electrically isolated conducting paths and it is required that the conducting paths are cut after the plating. For that purpose, the interval between the conducting paths whereby parts actually can be mounted cannot be made smaller than 400  $\mu\text{m}$ . Therefore, when gold electroplating is employed, the wiring density for semiconductor chips is decreased due to the presence of the conducting paths for continuity, leading to a problem that the improvement in the packing density of semiconductor chips is limited. Further, if the above electroless plating solution containing cyanide ions is used, although the above problem involved in the electroplating can be solved, gold is also liable as described above to deposit on a part of the insulator between conducting paths where the interval between the conducting paths is small. In particular, this phenomenon takes place noticeably in the case of a circuit board having surface conducting paths whose interval is 200  $\mu\text{m}$  or below. Therefore, when the above electroless gold plating solution containing cyanide ions is applied for the production of a circuit board having surface conducting paths whose interval is 200  $\mu\text{m}$  or below, the yield becomes poor. The above electroless gold plating solutions containing no cyanide ions are also unstable, and they are impossible to be applied to the mass production of a circuit board having surface conducting paths whose interval is 200  $\mu\text{m}$  or below, for the similar reason to the above electroless gold plating solution containing cyanide ions.

**SUMMARY OF THE INVENTION**

The first object of the invention is to provide an electroless gold plating solution capable of plating conducting paths whose interval is very small without causing gold to short-circuit the conducting paths, characterized in that the plating solution components contain no cyanide ions, and the amount of a reducing agent used is small.

The second object of the invention is to provide a method of electroless plating free from any safety problems in the plating operation and in the treatment of its waste solution.

The third object of the invention is to provide an electronic device on which parts can be mounted highly densely, and whose joint reliability to the parts is high.

The fourth object of the invention is to provide a module on which parts can be mounted highly densely, and whose joint reliability to the parts is high.

The fifth object of the invention is to provide a circuit board on which parts can be mounted highly densely, and joint reliability to the parts is high.

The sixth object of the invention is to provide a leadless chip carrier excellent in solderability.

The seventh object of the invention is to provide a tape carrier, the bonding strength of the conducting paths on the tape to electronic elements being high, and the efficiency of the utilization of the base film of the tape also being high.

The eighth object of the invention is to provide an X-ray lithography mask high in dimensional accuracy.

The above first object is achieved by providing an electroless gold plating solution comprising an aqueous solution that contains monovalent gold ions, a complexing agent which has a greater bond energy to the monovalent gold ions than hydroxide ions have, and a reducing agent.

The above second object is achieved by providing a method of plating with gold by using the above electroless gold plating solution according to the invention.

The above third to eighth objects are achieved by providing an electronic device, a module, a circuit board, a leadless chip carrier, a tape carrier, and an X-ray lithography mask that are plated with gold by using the above electroless gold plating solution.

The reason why the composition of the present electroless gold plating solution has been defined as described above is based on the following. The reason why a large amount of cyanide ions is used in the prior electroless gold plating solution is that the precipitation of gold which will occur when the gold complex reacts with hydroxide ions present in the plating solution is prevented by the cyanide ions that can bond as complexing agent to monovalent gold ions to form a stable gold complex. However, even when the prior electroless gold plating solution containing cyanide ions is used, gold sometimes happens to precipitate on the surface of an insulator where gold essentially cannot precipitate, and therefore it could not have been said that the prior gold plating solution containing cyanide ions is stable enough to be practical. The inventors considered that this is due to the assumption that, although the bond strength of a cyanide ion to a monovalent gold ion is considerably great, the bond strength is not so strong as the bond strength of a hydroxide ion to a monovalent gold ion. That is, it can be considered that since a hydroxide ion bonds more strongly to a monovalent gold ion than a cyanide ion does, gold hydroxide or gold oxide resulting therefrom precipitates. Further, when the precipitate adheres to the insulator surface, and gold precipitates thereon, a gold film may be formed even on the insulator surface. Even in the case wherein the prior electroless gold plating solution contains no cyanide ions, it is considered that the bond energy of the complexing agent used therein to a gold ion is smaller than that of a hydroxide ion, and therefore, a gold film is liable to be formed on the insulator surface, and the electroless gold plating solution is also not practical. In order to obtain a practical electroless gold plating solution, a complexing agent which has a greater bond strength to a monovalent gold ion than a hydroxide ion has must be found, but it is very difficult to find such a preferable complexing agent from countless compounds. Therefore, the inventors have used the molecular orbital method in quantum chemistry to determine chemical bond strengths theoretically, thereby finding excellent complexing agents. As a calculating method, the "ab initio SCF method" that is currently considered the most accurate has been adopted.

First, the origin of the strength of the bond between a monovalent gold ion and a cyanide ion that has hitherto been considered most strong has been studied. As a result it has been found that, in the interaction between a gold ion and a cyanide ion, there is only  $\sigma$  electron transfer from the cyanide ion to the gold ion, and there is little  $\pi$  electron transfer. Therefore, the inventors have judged that, as a ligand that can be substituted for a cyanide ion, a strongly  $\sigma$  electron donative ligand is preferable.

With respect to 13 complexing agents including a cyanide ion that have been, from experience, considered strongly  $\sigma$  electron donative and are listed in Table 1, the bond energy to a monovalent gold ion has been studied, and the order of the bond energies given in Table 1 have been obtained.

TABLE 1

|    | Complexing agent | Bond energy (kcal/mol) |
|----|------------------|------------------------|
| 20 | $S_2O_4^{2-}$    | 274                    |
|    | $SO_3^{2-}$      | 270                    |
|    | $OH^-$           | 260                    |
|    | $SH^-$           | 197                    |
|    | $CN^-$           | 196                    |
|    | $Cl^-$           | 173                    |
|    | $I^-$            | 157                    |
|    | $SCN^-$          | 122                    |
|    | $NH_3$           | 65                     |
|    | $CNCH_3$         | 56                     |
|    | $NCCN_3$         | 53                     |
| 30 | $PH_3$           | 39                     |
|    | $CO$             | 19                     |

Herein, The bond energy was calculated as the difference between energies before and after the formation of the bond between a monovalent gold ion and a complexing agent. If the above difference of energies concerning a gold ion and a complexing agent in a vacuum can be determined experimentally, difference can be used as the bond energy. From the accuracy of the above method of computation, it be considered that the order of the levels of the bond energies does not change between that of the experimental values and that of the calculated values. The result of the calculation, that the bond energy of a hydroxide ion to a monovalent gold ion is greater than that of a cyanide ion to a monovalent gold ion supports that the prior electroless gold plating solution using cyanide ions is unstable, which shows the above calculation is appropriate.

Based on this result, although the bond energies described above do not take hydration effect into consideration, it is highly probable that the essence of the real system can be considered by using the bond energies described above.

Among the 12 complexing agents, complexing agents having higher bond energies to a monovalent gold ion than a hydroxide ion were a thiosulfate ion and a sulfite ion only. Therefore, the inventors have considered that a thiosulfate ion and a sulfite ion are the most preferable to be used in an electroless gold plating solution.

Further, among known reducing agents, the inventors have selected experimentally ones which are preferable when a thiosulfate ion or a sulfite ion is used as a complexing agent. As a result, we have found that when thiourea, or its derivative such as methylthiourea, N-methylthiourea, and N-ethylthiourea, or hydroquinone, or its derivative such as methylhydroquinone, and ethylhydroquinone is used as a reducing agent, an aqueous solution containing monovalent gold ions and thiosulfate ions or an aqueous solution containing monova-

lent gold ions and sulfite ions can constitute a stable electroless gold plating solution. The present electroless gold plating solution has been obtained based on the above finding.

Herein, monovalent gold ions can be introduced into the plating solution by using, as a gold source, a gold (I) complex salt other than dicyanoaurate (I) complex salts such as a thiosulfatoaurate (I) complex salt. A thiosulfatoaurate (I) complex salt is a complex salt containing at least one thiosulfate ion around a gold atom per molecule. For example, dithiosulfatoaurate (I) can be mentioned and the molecular formula therefor is  $M_3[Au(S_2O_3)_3]$ , wherein M represents an alkali metal, for example M<sub>3</sub> may represent  $Na_2K$ . Further, a monovalent gold ion can be formed in an aqueous solution containing a mixture of a tetrahalogenoaurate (III) and a thiosulfate, so that that aqueous solution can be used. The molecular formula for a tetrahalogenoaurate (III) is  $MAuX_4$  wherein M represents an alkali metal such as Na, and K, and X represents a halogen atom such as F, and Cl, and as an example of a tetrahalogenoaurate (III) can be mentioned a tetrachloroaurate (III). A thiosulfate can be represented for example by  $M_2S_2O_3$  wherein M represents an alkali metal such as Na, and K. Since the thiosulfate ion or a sulfite ion is produced in an aqueous solution of a thiosulfate or a sulfite, a thiosulfate or a sulfite may be considered as a complexing agent.

The electroless gold plating solution according to the present invention has characteristics as mentioned above. By forming a gold coating film on an electronic device, a module, a circuit board, a leadless chip carrier, a tape carrier, and an X-ray lithography mask, the present electroless gold plating solution exhibits an excellent effect that has not been expected from the prior gold plating.

#### BRIEF DESCRIPTION OF THE DRAWINGS

FIG. 1 is a graph showing the relationship between the thickness ( $\mu m$ ) of gold coating and the plating time (h) obtained when gold was deposited by using an electroless gold plating solution of the present invention.

FIG. 2 is a flow chart of an example of a process of applying electroless gold plating onto a copper plate, showing a plating method of successively laminating a nickel film by electroplating, a gold film by electroplating, and a gold film by electroless plating.

FIG. 3 is a flow chart of an example of a process of applying electroless gold plating onto a copper plate, showing a plating method of successively laminating a nickel film by electroless plating, and a gold film by electroless plating.

FIG. 4 is a flow chart of an example of a process of applying electroless gold plating onto a copper plate, showing a plating method of successively laminating a gold film formed by sputtering and a gold film by electroless plating.

FIG. 5 is a flow chart of an example of a process of applying electroless gold plating onto a copper plate, showing a plating method of successively laminating a gold film formed by vacuum deposition, and a gold film by electroless plating.

FIG. 6 is a flow chart of an example of a process of applying electroless gold plating onto the surface of tungsten wires, showing a plating method of successively laminating a nickel film by electroless plating, a gold film by displacement plating, and a gold film by electroless plating on the surface of the tungsten wires

after the surface of the tungsten wires has been activated by a palladium activating solution.

FIG. 7 is a flow chart of an example of a process of applying electroless gold plating onto molybdenum wires, showing a plating method of successively laminating a nickel film by electroless plating, a gold film by displacement plating, and a gold film by electroless plating on the surface of the molybdenum wires after the surface of the molybdenum wires has been activated by a palladium activating solution.

FIG. 8 is a flow chart of an example of a process of applying electroless gold plating onto tungsten wires, showing a plating method of successively laminating a cobalt film by electroless plating, a gold film by displacement plating, and a gold film by electroless plating on the surface of the tungsten wires after the surface of the tungsten wires has been activated by a palladium activating solution.

FIG. 9 is a flow chart of an example of a process of applying electroless gold plating onto copper wires, showing a plating method of successively laminating a nickel film by electroless plating, a gold film by displacement plating, and a gold film by electroless plating on the surface of the copper wires after the surface of the copper wires has been activated by a palladium activating solution.

FIG. 10 is a perspective view of a ceramic circuit board plated with gold by using an electroless gold plating solution according to the invention.

FIG. 11 is a sectional view taken along line A—A of FIG. 10.

FIG. 12 (a) is a plan view of a ceramic circuit board and a printed circuit board plated with gold by using an electroless plating solution according to the present invention, and FIG. 12 (b) is a sectional view taken along line A—A of FIG. 12 (a).

FIG. 13 is a sectional perspective view of a module having a circuit board plated with gold by using an electroless gold plating solution according to the present invention.

FIG. 14 is a sectional view of the module of FIG. 13, showing mainly the multi-layer ceramic circuit board.

FIG. 15 is a sectional view, on an enlarged scale, of part of the surface conducting paths of the multi-layer ceramic circuit board of the module of FIG. 13.

FIG. 16 is a plan view of part of the first principal plane of the above multi-layer ceramic circuit board.

FIG. 17 is a partially sectional view of an electronic device having electronic elements mounted directly on a printed circuit board, with electroless gold plating according to the invention having been applied to the electronic device.

FIG. 18 is a sectional view of the surface conducting paths of the printed circuit board of FIG. 17.

FIG. 19 (a) is a perspective view of a leadless chip carrier plated with gold by using an electroless plating solution according to the present invention, and FIG. 19 (b) is a sectional view taken along line B—B of FIG. 19 (a).

FIG. 20 (a) is a plan view of the leadless chip carrier of FIG. 19, and FIG. 20 (b) is a bottom view of the leadless chip carrier of FIG. 19.

FIG. 21 is a plan view of a ceramic circuit board wherein a plurality of leadless chip carriers and conducting paths for their electroplating are formed together.

FIG. 22 is an enlarged view of a through-hole section of the above leadless chip carrier.

FIG. 23 is a plan view of a tape carrier plated with gold by using an electroless gold plating solution according to the invention.

FIG. 24 is a cross-sectional view of the tape carrier of FIG. 23.

FIG. 25 is a view showing the layer structure of the film on the copper wires of the above tape carrier.

FIG. 26 is a cross-sectional view of an X-ray lithography mask plated with gold by using an electroless gold plating solution according to the invention.

FIG. 27 is a chart showing the manufacturing process of the above X-ray lithography mask.

#### DETAILED DESCRIPTION OF THE PREFERRED EMBODIMENTS

The present invention will now be described in detail by the following examples.

#### EXAMPLE 1

A nickel coating having a thickness of 2  $\mu\text{m}$  was formed on each copper plate 2.5 cm by 2.5 cm by 0.3 mm by the process shown in FIG. 2 using a usual nickel electroplating solution, and then a gold coating having a thickness of 1  $\mu\text{m}$  was formed thereon by using a usual gold electroplating solution to obtain a sample. The samples were degreased, then washed with dilute hydrochloric acid, and washed with water well. After the samples were dried by nitrogen gas blow, the samples were weighed. The samples were immersed for 2 hours in electroless gold plating solutions according to the invention that had the formulations shown below under the plating conditions shown below.

-continued

| Formulations of the electroless gold plating solutions and plating conditions |         |
|-------------------------------------------------------------------------------|---------|
| 5                                                                             | pH 10.0 |

Each of the above plating solutions was stirred forcibly, and every 30 minutes the sample was taken out, and the gold film thickness was determined by the gravimetric method. The results are given in FIG. 1 as curves 1-5 that correspond to (a) to (e) above. The deposited gold film in any of the cases using the above plating solutions had a mat bright yellow color, and no precipitation was observed in any of the plating solutions.

10 Deposition rates and the presence of a precipitation in the plating solutions having formulations outside the above formulations were examined under plating conditions outside the above plating conditions, and preferable ranges of the amounts of components in the formulations and plating conditions were obtained as shown below.

15 (1) The amount of the dithiosulfatoaurate (I) complex salt was favorably 0.001 to 0.2 mol/l, preferably 0.006 to 0.04 mol/l, and particularly preferably 0.01 to 0.03 mol/l. If the amount was less than 0.001 mol/l, the reaction became slow, whereas if the amount was more than 0.2 mol/l, a precipitation of gold occurred in the plating solution.

20 (2) When a mixture of the tetrahalogenoaurate (III) and the thiosulfate was used as a source of gold, the amount of the tetrahalogenoaurate (III) was favorably 0.001 to 0.2 mol/l, preferably 0.006 to 0.05 mol/l, and particularly preferably 0.01 to 0.03 mol/l. If the amount was less than 0.001 mol/l, the reaction became slow, whereas if the amount was more than 0.2 mol/l, a precipitation of gold occurred in the plating solution.

25 (3) The amount of the reducing agent was favorably 0.001 to 1.0 mol/l, preferably 0.01 to 0.5 mol/l, and particularly preferably 0.02 to 0.3 mol/l. If the amount was less than 0.001 mol/l, the reaction became slow, whereas if the amount was more than 1.0 mol/l, the effect on the plating was not specially improved, and the excess amount of the reducing agent was wasteful.

30 (4) The amount of the thiosulfate was favorably 0.001 to 0.9 mol/l, and if the thiosulfatoaurate (I) complex salt was used as a gold source, the amount is preferably 0.01 to 0.4 mol/l, and particularly preferably 0.05 to 0.1 mol/l. If the tetrahalogenoaurate (III) was used as a gold source, the amount was preferably 0.003 to 0.6 mol/l, and particularly preferably 0.04 to 0.2 mol/l. If the amount was less than 0.001 mol/l, a precipitation of gold likely occurred, whereas if the amount was more than 0.9 mol/l, a precipitation of sulfur occurred.

35 (5) The amount of the sulfite as a stabilizer was favorably 0.01 to 0.8 mol/l, preferably 0.08 to 0.7 mol/l, and particularly preferably 0.15 to 0.5 mol/l. If the amount was less than 0.01 mol/l, a precipitation of sulfur likely occurred, whereas if the amount was more than 0.8 mol/l, the reaction of the plating became slow.

40 (6) The amount of the pH adjuster was favorably 0.09 to 1.0 mol/l, preferably 0.4 to 1.0 mol/l, and particularly preferably 0.4 to 0.8 mol/l. If the amount was less than 0.09 mol/l, the deposition rate became reduced after the start of the plating reaction, whereas if the amount was more than 1.0 mol/l, the effect on the plating was not specially improved, and the pH adjuster became wasteful.

| Formulations of the electroless gold plating solutions and plating conditions |             |
|-------------------------------------------------------------------------------|-------------|
| (a) Sodium dithiosulfatoaurate (I)                                            | 0.02 mol/l  |
| Sodium thiosulfate                                                            | 0.2 mol/l   |
| Thiourea                                                                      | 0.2 mol/l   |
| Sodium sulfite                                                                | 0.2 mol/l   |
| Ammonium chloride                                                             | 0.2 mol/l   |
| Water                                                                         | 1 l         |
| Solution temperature                                                          | 60° C.      |
| pH                                                                            | 7.0         |
| (b) Sodium dithiosulfatoaurate (I)                                            | 0.02 mol/l  |
| Sodium thiosulfate                                                            | 0.25 mol/l  |
| Thiourea                                                                      | 0.1 mol/l   |
| Sodium sulfite                                                                | 0.2 mol/l   |
| Ammonium chloride                                                             | 0.2 mol/l   |
| Water                                                                         | 1 l         |
| Solution temperature                                                          | 80° C.      |
| pH                                                                            | 8.5         |
| (c) Sodium dithiosulfatoaurate (I)                                            | 0.05 mol/l  |
| Sodium thiosulfate                                                            | 0.5 mol/l   |
| N-methylthiourea                                                              | 0.1 mol/l   |
| Sodium sulfite                                                                | 1.0 mol/l   |
| Sodium tetraborate                                                            | 0.1 mol/l   |
| Water                                                                         | 1 l         |
| Solution temperature                                                          | 70° C.      |
| pH                                                                            | 8.0         |
| (d) Sodium tetrachloroaurate (III)                                            | 0.025 mol/l |
| Sodium thiosulfate                                                            | 0.25 mol/l  |
| Hydroquinone                                                                  | 0.04 mol/l  |
| Sodium sulfite                                                                | 0.3 mol/l   |
| Sodium tetraborate                                                            | 0.1 mol/l   |
| Water                                                                         | 1 l         |
| Solution temperature                                                          | 80° C.      |
| pH                                                                            | 9.0         |
| (e) Sodium tetrachloroaurate (III)                                            | 0.025 mol/l |
| Sodium thiosulfate                                                            | 0.1 mol/l   |
| Methylhydroquinone                                                            | 0.05 mol/l  |
| Sodium sulfite                                                                | 0.4 mol/l   |
| Sodium tetraborate                                                            | 0.2 mol/l   |
| Water                                                                         | 1 l         |
| Solution temperature                                                          | 70° C.      |

(7) The solution temperature was 60° to 90° C., preferably 65° to 85° C., and particularly preferably 70° to 80° C. If the solution temperature was lower than 60° C., the plating reaction became slow, whereas if the solution temperature was higher than 90° C., a precipitation occurred in the plating solution.

(8) The pH of the plating solution was favorably 7.0 to 11.0, preferably 7.5 to 10.0, and particularly preferably 8.0 to 9.0. If the pH was lower than 7.0, the plating reaction became slow, whereas if the pH was higher than 11.0, a precipitation occurred in the plating solution.

#### EXAMPLE 2

Samples prepared in the same way as those in Example 1 were immersed in an electroless gold plating solution having the following composition according to the invention under the following plating conditions. In this Example, as a complexing agent, sodium sulfite was used.

Composition of the electroless gold plating solution and the plating conditions

|                                |            |
|--------------------------------|------------|
| Sodium dithiosulfatoaurate (I) | 0.02 mol/l |
| Sodium sulfite                 | 0.5 mol/l  |
| Thiourea                       | 0.2 mol/l  |
| Sodium tetraborate             | 0.08 mol/l |
| Water                          | 1 l        |
| Solution temperature           | 90° C.     |
| pH                             | 8.0        |

The above plating solution was stirred forcibly, and after two hours, the thickness of the gold film was measured by the gravimetric method. The thickness of the gold film was 2.1  $\mu$ m. The deposited gold film was mat and bright yellow, and no precipitation was observed in the plating solution. The deposition rate and the presence of precipitation in the plating solution was examined using amounts of sodium sulfite outside the above amount, and a preferable range of the amount of the sulfite given below was obtained. The amount of the sulfite as a complexing agent was favorably 0.005 to 0.5 mol/l, preferably 0.03 to 0.4 mol/l, and particularly preferably 0.05 to 0.3 mol/l. If the amount was less than 0.005 mol/l or more than 0.5 mol/l, a precipitation of gold was likely to occur.

#### EXAMPLE 3

A nickel film having a thickness of 2  $\mu$ m and then a gold film having a thickness of 1  $\mu$ m were formed by the process shown in FIG. 3 on a copper plate 2.5 cm  $\times$  2.5 cm  $\times$  0.3 mm to prepare a sample. After the sample was pretreated in the same way as Example 1, the sample was immersed in the present electroless gold plating solution having the composition shown in (e) above in Example 1 under the plating conditions shown in (e) in Example 1. The plating solution was forcibly stirred, and after two hours the thickness of the gold film was measured by the gravimetric method. The thickness of the gold film was 1.2  $\mu$ m. The deposited gold film was slightly lustrous bright yellow, and no precipitation was observed in the plating solution.

#### EXAMPLE 4

A gold film having 2000  $\text{\AA}$  thickness was formed on a copper plate 2.5 cm  $\times$  2.5 cm  $\times$  0.3 mm by the process shown in FIG. 4 using a usual sputtering unit to prepare a sample. After the sample was pretreated in the same way as Example 1, the sample was immersed in the

present electroless gold plating solution having the composition shown in (e) in Example 1 under the plating conditions shown in (e) in Example 1. The plating solution was forcibly stirred, and after two hours the thickness of the gold film was measured by the gravimetric method. The thickness of the gold film was 1.3  $\mu$ m. The deposited gold film was mat and bright yellow, and no precipitation was observed in the plating solution.

#### EXAMPLE 5

A gold film having a thickness of 1000  $\text{\AA}$  was formed by the process shown in FIG. 5 using a usual metallizing apparatus on a copper plate 2.5 cm  $\times$  2.5 cm  $\times$  0.3 mm to prepare a sample. After the sample was pretreated in the same way as Example 1, the sample was immersed in the present electroless gold plating solution having the composition shown in (b) in Example 1 under the plating conditions shown in (b) in Example 1. The plating solution was forcibly stirred, and after two hours the thickness of the gold film was measured by the gravimetric method. The thickness of the gold film was 1.5  $\mu$ m. The deposited gold film was mat, and bright yellow, and no precipitation was observed in the plating solution.

#### EXAMPLE 6

Each alumina ceramic board plated with gold using an electroless gold plating solution according to the invention is shown in FIG. 10 and a sectional view thereof is shown in FIG. 11. The surface of each conductor of a die bonding pad 7 of tungsten, wire bonding pads 8 of tungsten, and leads 9 of Kovar® was plated by the plating process shown in FIG. 6. After each conductor was activated by a usual palladium activator, a nickel film having a thickness of 3  $\mu$ m was formed thereon by using a usual electroless nickel plating solution, and then a gold film having a thickness of 0.3  $\mu$ m was formed by using a usual displacement gold plating solution. The board was washed with a decreasing solution and then with dilute hydrochloric acid, and then was dried by nitrogen gas blow. Then the board was immersed for 3 hours in the electroless gold plating solution according to the present invention having the composition shown in (a) in Example 1 under the plating conditions shown therein, and the plating solution was stirred forcibly. The deposited gold film had a thickness of 1.8  $\mu$ m.

20 ceramic boards thus prepared were used as samples, and the joining properties of the gold plated parts thereof were assessed as follows.

##### (1) Die-bonding Property

After die-bonding of the die-bonding pad and the silicon chip was carried out at 430° C. in a nitrogen atmosphere by a usual method, a heat shock test (0° C.  $\leftrightarrow$  200° C., 5 cycles with each cycle for 10 sec) was carried out, and one wherein the silicon chip did not come off was assessed as good one.

##### (2) Wire Bonding Property

After a gold wire having a diameter of 25  $\mu$ m was pressed to be in contact with the wire bonding pad 8 of the sample heated to about 150° C., the wire was pulled by applying a load of 6 g, and one wherein the wire did not come off from the wire bonding pad 8 was assessed as a good one.

## (3) Solderability

After the sample was heated at 460° C. for 15 min in air, the leads 9 were immersed in solder, and one wherein 95% or over of the lead area was wetted with the solder was assessed as a good one.

As a result of the above assessment, all of the 20 samples were assessed as good ones. Therefore, when electroless gold plating solutions according to the present invention are used, a ceramic circuit board having conducting paths of tungsten and excellent in joining properties can be obtained in a safe working environment.

## EXAMPLE 7

The present electroless gold plating solution was applied to each alumina ceramic board 6 that was the same as shown in Example 6 except that the die-bonding pad 7 and the wire bonding pads 8 were made of molybdenum, and the plating process shown in FIG. 7 was applied. The board was subjected to activation, nickel plating, and displacement gold plating in the same way as in Example 6, and then was immersed for 3 hours in the electroless gold plating solution having the composition shown in (a) in Example 1 under the plating conditions shown therein, and the plating solution was stirred forcibly. The thickness of the deposited gold film was 1.7  $\mu\text{m}$ . The thus formed 20 ceramic boards were used as samples, and the joining properties of the gold plated parts thereof were assessed in the same way as in Example 6. All of the 20 samples were assessed as good ones. Therefore, when electroless gold plating solutions according to the present invention are used, a ceramic circuit board having conducting paths of molybdenum and excellent in joining properties can be obtained in a safe working environment.

## EXAMPLE 8

20 ceramic circuit boards each having on an alumina ceramic 11 a wiring pattern 10 that is shown in FIG. 12 and was made of tungsten conductor, with the interval between the conducting paths being varied for each group of 20, were prepared. Specifically, 20 ceramic circuit boards with the interval between the conducting paths being 300  $\mu\text{m}$ , 20 similar ceramic circuit boards with the interval between the conducting paths being 200  $\mu\text{m}$ , 20 similar ceramic circuit boards with the interval between the conducting paths being 100  $\mu\text{m}$ , and 20 similar ceramic boards with the interval between the conducting paths being 30  $\mu\text{m}$  were prepared. The boards were plated by using the plating process shown in FIG. 6. After the tungsten surface constituting the wiring pattern 10 was activated by a usual palladium activator, a nickel film having a thickness of 5  $\mu\text{m}$  was formed by using a usual electroless nickel plating solution, and thereon displacement plating was carried out by using a usual displacement gold plating solution. The thicknesses of the gold films on all the boards were measured by an X-ray fluorescence coating thickness gauge and were found to be 0.2 to 0.4  $\mu\text{m}$ . 10 samples of each of the four types different in the interval between the conducting paths were plated by using an electroless gold plating solution having the following composition under the following conditions.

| Composition of the plating solution and plating conditions |            |
|------------------------------------------------------------|------------|
| Sodium tetrachloroaurate (III)                             | 0.01 mol/l |

-continued

| Composition of the plating solution and plating conditions |            |
|------------------------------------------------------------|------------|
| Sodium thiosulfate                                         | 0.08 mol/l |
| Thiourea                                                   | 0.05 mol/l |
| Sodium sulfite                                             | 0.4 mol/l  |
| Sodium tetraborate                                         | 0.1 mol/l  |
| Water                                                      | 1 l        |
| Solution temperature                                       | 80° C.     |
| pH                                                         | 9.0        |

10

15

20

25

30

35

40

45

50

55

60

65

70

75

80

85

90

95

100

105

110

115

120

125

130

135

140

145

150

155

160

165

170

175

180

185

190

195

200

205

210

215

220

225

230

235

240

245

250

255

260

265

270

275

280

285

290

295

300

305

310

315

320

325

330

335

340

345

350

355

360

365

370

375

380

385

390

395

400

405

410

415

420

425

430

435

440

445

450

455

460

465

470

475

480

485

490

495

500

505

510

515

520

525

530

535

540

545

550

555

560

565

570

575

580

585

590

595

600

605

610

615

620

625

630

635

640

645

650

655

660

665

670

675

680

685

690

695

700

705

710

715

720

725

730

735

740

745

750

755

760

765

770

775

780

785

790

795

800

805

810

815

820

825

830

835

840

845

850

855

860

865

870

875

880

885

890

895

900

905

910

915

920

925

930

935

940

945

950

955

960

965

970

975

980

985

990

995

1000

1005

1010

1015

1020

1025

1030

1035

1040

1045

1050

1055

1060

1065

1070

1075

1080

1085

1090

1095

1100

1105

1110

1115

1120

1125

1130

1135

1140

1145

1150

1155

1160

1165

1170

1175

1180

1185

1190

1195

1200

1205

1210

1215

1220

1225

1230

1235

1240

1245

1250

1255

1260

1265

1270

1275

1280

1285

1290

1295

1300

1305

1310

1315

1320

1325

1330

1335

1340

1345

1350

1355

1360

1365

1370

1375

1380

1385

1390

1395

1400

1405

1410

1415

1420

1425

1430

1435

1440

| Composition of the palladium activator |         |
|----------------------------------------|---------|
| Water                                  | 1 l     |
| Palladium chloride                     | 0.2 g/l |
| Hydrochloric acid                      | 50 ml/l |

Thereafter, a nickel film having a thickness of 5  $\mu\text{m}$  was formed by using a usual electroless nickel plating solution, and thereon displacement gold plating was carried out by using a usual displacement gold plating solution. The thicknesses of the gold films on all the boards were measured by an X-ray fluorescence coating thickness gauge and were found to be 0.2 to 0.3  $\mu\text{m}$ . 10 samples of each of the four types of the boards different in the interval between the conducting paths were plated with gold by using an electroless gold plating solution having the following composition.

| Composition of the plating solution and plating conditions |            |
|------------------------------------------------------------|------------|
| Sodium dithiosulfatoaurate (I)                             | 0.02 mol/l |
| Sodium thiosulfate                                         | 0.20 mol/l |
| Thiourea                                                   | 0.15 mol/l |
| Sodium sulfite                                             | 0.2 mol/l  |
| Ammonium chloride                                          | 0.1 mol/l  |
| Water                                                      | 1 l        |
| Solution temperature                                       | 80° C.     |
| pH                                                         | 8.0        |

For comparison the remaining boards were plated with gold by using a usual electroless gold plating solution containing no cyanide ions similarly to Example 8. After the plating, the thicknesses of the gold films were measured, and in the case using the plating solution having the above composition, the thicknesses were 1.7 to 2.0  $\mu\text{m}$ , whereas in the case using the above commercially available plating solution, the thicknesses were 1.6 to 1.8  $\mu\text{m}$ . The surfaces of the thus prepared printed circuit boards were observed by an optical microscope, and assessment was made such that if of 10 circuit boards there were 2 or more circuit boards wherein gold deposited between the conducting paths of the wiring pattern 10 to form a short circuit, they were judged to be defective, and if of 10 circuit boards there was 0 or 1 circuit board wherein gold deposited between the conducting paths of the wiring pattern 10 to form a short circuit, the circuit board was judged to be good. The results are shown in Table 3.

TABLE 3

| Interval between conducting paths ( $\mu\text{m}$ ) | Plating solution according to the invention | Usual plating solution |
|-----------------------------------------------------|---------------------------------------------|------------------------|
| 300                                                 | good                                        | good                   |
| 200                                                 | good                                        | defective              |
| 100                                                 | good                                        | defective              |
| 30                                                  | good                                        | defective              |

Thus when an electroless gold plating solution according to the invention is used, a gold film having a thickness of 0.5  $\mu\text{m}$  or over can be formed on a surface wiring system on a printed circuit board with the interval between the conducting paths being 200  $\mu\text{m}$  or below by plating, and therefore a printed circuit board on which parts can be mounted highly densely can be produced. Moreover, a short circuit due to deposition of gold on the insulator surface of the board would not occur.

## EXAMPLE 10

This is an example wherein gold plating by using an electroless gold plating solution according to the invention was applied to a multi-layer ceramic circuit board 12 of a module shown in FIG. 13. The multi-layer ceramic circuit board 12 had a structure shown in FIG. 14, and consisted of a ceramic insulator 16 and tungsten conducting paths 12. On the first principal plane of the board, there are chip joining pads 18 to which semiconductor chips 13 will be joined by soldering, engineering change pads 19 where wire bonding for wiring alteration will be made, and sealing pads 20 where caps 15 for seal into which a refrigerant will be passed will be soldered, and on the second principal plane, there are brazing pads 21 for pins where I/O pins 14 will be brazed. Connections by soldering, wire bonding, or brazing will be made to these tungsten surface conducting paths, so that the tungsten 22 is covered with a nickel film 23, and then a gold film 24 as shown in FIG. 15.

Five types of multi-layer ceramic circuit boards were prepared, that is, ones wherein the interval A between chip joining pads 18 (shown in FIG. 16) was 10  $\mu\text{m}$ , ones wherein the interval A between chip joining pads 18 (shown in FIG. 16) was 50  $\mu\text{m}$ , ones wherein the interval A between chip joining pads 18 (shown in FIG. 16) was 100  $\mu\text{m}$ , ones wherein the interval A between chip joining pads 18 (shown in FIG. 16) was 200  $\mu\text{m}$ , and ones wherein the interval A between chip joining pads 18 (shown in FIG. 16) was 400  $\mu\text{m}$ , were prepared. For each type of the above five types where the intervals between the conducting paths were different, 10 multi-layer ceramic boards whose major component was alumina, and 10 multi-layer mullite ceramic boards whose major component was mullite, were prepared. After tungsten constituting the surface wiring system of each board was activated by a usual palladium activator, a nickel film having a thickness of 5  $\mu\text{m}$  was formed thereon by using a usual electroless nickel plating solution, and then gold plating was made thereon by using a usual displacement gold plating solution. The thicknesses of the gold films on circuit boards whose major component was alumina and circuit boards whose major component was mullite were measured by an X-ray fluorescence coating thickness gauge, and were found to be 0.1 to 0.3  $\mu\text{m}$ . These boards were plated with gold by using an electroless gold plating solution according to the invention having the following composition under the following plating conditions.

| Composition of the plating solution and plating conditions |             |
|------------------------------------------------------------|-------------|
| Sodium tetrachloroaurate (III)                             | 0.015 mol/l |
| Sodium thiosulfate                                         | 0.1 mol/l   |
| Thiourea                                                   | 0.04 mol/l  |
| Sodium sulfite                                             | 0.3 mol/l   |
| Sodium tetraborate                                         | 0.1 mol/l   |
| Water                                                      | 1 l         |
| Solution temperature                                       | 80° C.      |
| pH                                                         | 9.0         |

The above plating solution was stirred forcibly, and after plating for 2 hours, the thicknesses of the deposited gold films were measured, and in either case wherein the major component of the circuit boards was alumina and case wherein the major component of the circuit boards was mullite, the thicknesses of the gold films were 2.0 to 2.3  $\mu\text{m}$ . For comparison, multi-layer ce-

ramic circuit boards were plated for 2 hours in the same way as above, except that, as the electroless gold plating solution, a usual electroless gold plating solution containing cyanide ions was used. The thicknesses of the deposited gold films were measured, and in either case wherein the major component of the circuit board was alumina and case wherein the major component of the circuit board was mullite, the thicknesses were 1.8 to 2.0  $\mu\text{m}$ . The surfaces of the thus prepared multi-layer ceramic circuit boards were observed by an optical microscope to examine whether there was a short circuit due to the deposition of gold on the insulator surface. With respect to 10 multi-layer ceramic circuit boards of each of five types whose major component was alumina and that had a certain interval between the conducting paths, and 10 multi-layer ceramic boards of each of five types whose major component was mullite and that had a certain interval between the conducting paths, the numbers of boards wherein a short circuit was observed are shown in Table 4. In all of the circuit boards plated with gold by using the present electroless gold plating solution, any short circuit was not found at all.

TABLE 4

| Interval between conducting paths ( $\mu\text{m}$ ) | Multi-layer ceramic circuit board whose major component was alumina |                        | Multi-layer ceramic circuit board whose major component was mullite |                        |
|-----------------------------------------------------|---------------------------------------------------------------------|------------------------|---------------------------------------------------------------------|------------------------|
|                                                     | Plating solution according to the invention                         | Usual plating solution | Plating solution according to the invention                         | Usual plating solution |
| 400                                                 | 0                                                                   | 0                      | 0                                                                   | 0                      |
| 200                                                 | 0                                                                   | 4                      | 0                                                                   | 5                      |
| 100                                                 | 0                                                                   | 10                     | 0                                                                   | 10                     |
| 50                                                  | 0                                                                   | 10                     | 0                                                                   | 10                     |
| 10                                                  | 0                                                                   | 10                     | 0                                                                   | 10                     |

Then, using circuit boards wherein any short circuit was not observed, modules were assembled as shown in FIG. 13. Semiconductor chips 13 were soldered, wire bonding was made to engineering change pads 19, and caps 15 for seal were soldered. I/O pins 14 were joined by using gold-germanium brazing filler metal.

The joined sections of the assembled modules were checked as follows. With respect to the soldering of the semiconductor chips, the wire bonding, and the brazing of I/O pins, electrical check was carried out by passing an electric signal to all the joined sections. With respect to the soldering of the sealed sections, after the inside of each of the modules was filled with helium gas, and then was made gas-tight, the module was placed in a container that has been evacuated thereby examining whether there was a leak of the helium gas. Thus, with respect to all the assembled modules, it has been confirmed that there were no defective joining of the semiconductor chips, and no defective wire bonding, and there was no leak of the helium gas at the sealed sections, which showed no defective joining of the sealed sections.

With respect to each of the assembled modules, the delay property of an electric signal due to the board was measured. Thus it was found that the signal delay due to the circuit boards having an interval of 50  $\mu\text{m}$  between the conducting paths obtained by using the present electroless gold plating solution was about  $\frac{1}{2}$  of that of the circuit boards having an interval of 200  $\mu\text{m}$  between the conducting paths that was minimum when the usual electroless gold plating solution was used.

Thus, by plating a board of a module with gold by using an electroless gold plating solution according to the invention, a board on which parts can be mounted highly densely, and wherein the joint reliability is high can be produced in a high yield. Consequently, a module wherein the electric signal delay due to the board is small can be produced. In particular, when the present electroless gold plating solution is applied to gold plating of a board of a module for electronic computers, parts can be mounted more densely than in the case wherein a usual electroless gold plating solution is applied, and a module wherein the electric signal delay due to the board is less can be produced in a high yield, so that the present invention is effective for the mass production of high-speed electronic computers.

## EXAMPLE 11

A copper-clad laminate 25 (the substrate being glass-epoxy resin) was used to form a printed circuit board for a chip-on-board (COB) wherein semiconductor chips will be directly mounted without using a package onto the printed circuit board as shown in FIG. 17, and a conductor circuit was formed by a usual circuit forming method (subtract method). Then after other part than the wire bonding pad 26 in FIG. 17 was selectively masked by a dry film resist, the board was immersed in a palladium activating solution ( $\text{PdCl}_2$ : 0.2 g/l;  $\text{HCl}$ : 50 ml/l) to activate the conductor surface. Then, by using an electroless nickel plating solution, a displacement gold plating solution, and an electroless gold plating solution having the composition and plating conditions shown below, a nickel coating having a thickness of 1  $\mu\text{m}$  (32), and a gold coating having a thickness of 3  $\mu\text{m}$  (33) were formed on the bonding pad 26 (on copper). The resist was removed after the plating to form a printed circuit board having a bonding pad consisting of a metallized constitution as shown in FIG. 18.

## Composition of the electroless gold plating solution

|                     |            |
|---------------------|------------|
| Sodium chloroaurate | 0.01 mol/l |
| Sodium thiosulfate  | 0.1 mol/l  |
| Sodium sulfite      | 0.4 mol/l  |
| Sodium tetraborate  | 0.1 mol/l  |
| Thiourea            | 0.05 mol/l |

## Plating conditions

pH: 9.0  
Temperature: 80° C.

A semiconductor element (chip) 29 was joined onto the die-bonding pad 27 on the board by using a conductive epoxy adhesive (containing Ag). Then by using a thermionic bonder (bonding pressure: 100 g), gold wires having a diameter of 30  $\mu\text{m}$  were joined to the bonding pad of the semiconductor element 29 and the bonding pad 26 on the board. The joined states were assessed by tension test of the gold wires, and were found to be the tearing mode of the gold wires, and good bonding ability was confirmed.

## EXAMPLE 12

As shown in FIGS. 19 and 20, each leadless chip carrier formed with tungsten wires die-bonding pads 35, wire bonding pads 36, soldering pads 38, and through-holes 37) that were formed on an alumina ceramic board 34 by a usual method was plated according to the plating process shown in FIG. 6. First, the tungsten was activated by using a usual palladium activating solution, a nickel coating having a thickness of 4  $\mu\text{m}$  was formed

by using a usual electroless nickel plating solution, and then a gold coating having a thickness of 0.1  $\mu\text{m}$  was formed by using a usual displacement gold plating solution. 20 leadless chip carriers thus formed were immersed in the present electroless gold plating solution having the composition and plating conditions mentioned in Example 10 to form a gold coating having a thickness of 2  $\mu\text{m}$ .

Since the prior plating was carried out by using an electroplating solution, electroplating was also carried out for comparison. In this case, as shown in FIG. 21, conducting paths of leadless chip carriers 39 and conducting paths 40 for continuity between the conducting paths of leadless chip carriers were formed on each the same alumina ceramic boards followed by electroplating. Thereafter the conducting paths for continuity were broken and removed to form single leadless chip carriers. The electroplating was carried out as follows. A nickel coating having a thickness of 4  $\mu\text{m}$  was formed on the tungsten wires by using a usual nickel electroplating solution, and then a gold coating having a thickness of 2  $\mu\text{m}$  was formed thereon by using a usual gold electroplating solution. After the completion of the plating, the board was broken, and the single leadless chip carriers were taken out.

The thus-formed leadless chip carriers that had been subjected to the electroless plating and the thus-formed leadless chip carriers that had been subjected to the electroplating were assessed by steam aging described below. That is, about 1 l of pure water was boiled in a 2-l beaker, and each leadless chip carrier was placed about 3.8 mm over the water surface, and was allowed to stand for 1 hour with 7/8 of the opening of the beaker covered. One wherein the soldering pads 38 were not discolored, and when solder dipping was done to the 35 soldering pads 95% or over of the area of the soldering pads were wetted, was judged to be good. Thus, all 20 leadless chip carriers prepared by using the present electroless gold plating solution were judged to be good, whereas of 20 leadless chip carriers prepared by using the conventional electroplating process, only 3 leadless chip carriers were judged to be good.

This result will be attributed to the following reason. When an electroless gold plating according to the invention is applied, all the surface of conducting paths is covered with a gold coating free from any pinholes. On the other hand, if the conventional electroplating is carried out, a fracture of the through-hole 37 as shown in FIG. 22 will be formed by breaking and removing the conducting paths for continuity, resulting in the exposure of the nickel 42 and the tungsten 43 under the gold coating 41. These metals will be turned to oxides by the steam aging, and the oxides will spread to the soldering pad 38, causing defective wetting. Further, when the conventional electroless gold plating solution is used, the above problem will not occur, but gold is likely to deposit on the ceramic of the board of the leadless chip carrier, and the yield will become poor. Therefore, when the electroless gold plating solution of the present invention is applied to gold plating of a leadless chip carrier, a leadless chip carrier high in joint reliability can be produced in a high yield.

#### EXAMPLE 13

After tungsten wires were formed on each alumina 65 ceramic board 34 in a usual manner, each leadless chip carrier shown in FIGS. 19 and 20 was plated according to the plating process shown in FIG. 8. First, the tung-

sten was activated by using a usual palladium activating solution, a cobalt coating having a thickness of 4  $\mu\text{m}$  was formed by using a usual electroless cobalt plating solution, and then a gold coating having a thickness of 0.1  $\mu\text{m}$  was formed by using a usual displacement gold plating solution. 20 leadless chip carriers thus prepared were immersed in an electroless gold plating solution having the composition and plating conditions shown in Example 10 according to the invention to form a gold coating having a thickness of 2  $\mu\text{m}$ . In the same manner as in Example 12, electroplating was also carried out for comparison. The boards used were suitable for electroplating, and the same as used in Example 12 as shown in FIG. 21, and a cobalt coating having a thickness of 4  $\mu\text{m}$ , and a gold coating having a thickness of 2  $\mu\text{m}$ , were formed by using a usual cobalt electroplating solution, and a usual gold electroplating solution, respectively. The boards were broken to prepare 20 leadless carriers.

After these electroless plated leadless chip carriers, and electroplated leadless chip carriers were subjected to steam aging in the same way as Example 12, the wettability of the soldering pads 38 was assessed. All of 20 leadless chip carriers prepared by using the present electroless gold plating solution were judged to be good, whereas of 20 leadless chip carriers prepared by using the electroplating, only 4 leadless chip carriers were judged to be good. The cause was the same as that in Example 12. In the case where the conventional electroless gold plating solution was used, gold was liable to deposit on the ceramic, and the yield was poor. Therefore, by the plating process using the present electroless gold plating solution, a leadless chip carrier high in joint reliability can be produced in a high yield.

#### EXAMPLE 4

A tape carrier as shown in FIG. 23 was formed in the following steps. An insulating film 44 of polyimide or the like to which a copper foil having a thickness of 35  $\mu\text{m}$  was formed with sprocket holes 45 for feeding the tape. Then after a prescribed resist pattern was formed by a usual photo-process, the copper foil was etched with an etching solution containing ammonium persulfate or the like to form prescribed copper wires 46. Thereafter, the surface of the copper wires was activated by an activating solution containing palladium chloride and hydrochloric acid, and then a nickel coating 47 having a thickness of about 3  $\mu\text{m}$  was formed by using an electroless nickel plating solution containing nickel sulfate as a major component and sodium hypophosphite as a reducing agent. Then, a gold coating having a thickness of about 0.1  $\mu\text{m}$  was formed on the nickel coating by using a displacement gold plating solution containing potassium dicyanoaurate (I) as a major component. This gold coating was used as a catalyst to form a gold coating 48 having a thickness of about 1  $\mu\text{m}$  by using the above present electroless gold plating solution. The layer structure of the plated coatings formed on the above copper wires is shown in FIG. 24. As shown in FIG. 25, tips 49 of the copper wires of the tape carrier thus formed and bumps of gold formed on a semiconductor 50 were bonded by thermocompression. The bond strength was measured, and a tensile strength of 50 g or over per bump was obtained. This strength is twice or more as high as a tensile strength of about 20 g of the case wherein only replacement gold plating is carried out, that is, the thickness of gold is about 0.1  $\mu\text{m}$ .

To form a gold coating having a thickness of about 1  $\mu\text{m}$ , both a cyanide type electroless gold plating solution, and electroplating can be used. However, in the case of a cyanide type electroless gold plating, since the solution temperature is 90° C., and the pH is 13, a base film of polyimide or the like, and an adhesive bonding copper wires and the base film will be melted, so that the cyanide type electroless gold plating solution cannot be used. In the case of electroplating, since a pattern for electricity supply has to be formed, the efficiency of the utilization of the base film is decreased, and the cost becomes high.

#### EXAMPLE 15

An x-ray lithography mask according to the present invention and its manufacture will now be described.

FIG. 26 is a cross-sectional view of the constitution of an X-ray lithography mask according to the present invention. An X-ray transparent substrate 53 is formed on a mask board 52, for example, a silicon single crystal board. The X-ray transparent substrate 53 has a thickness of 0.5 to 5  $\mu\text{m}$ , and comprises a film of a high-temperature resin, such as polyimide, and polyimidoamide, and an inorganic compound and a metal having a higher X-ray transmission such as silicon oxide, silicon nitride, boron, and titanium. On the X-ray transparent substrate the X-ray absorption pattern 54 having a prescribed shape was formed by using the above present electroless gold plating solution. For the purpose of improving the adhesion between the X-ray absorption pattern and the X-ray transparent substrate, an underlay film 55 of nickel, copper or the like, and an adhesive layer 56 may be formed additionally.

Referring to FIG. 27, the process of production of the present X-ray lithography mask will now be described. (a) A mask board 52 such as a silicon wafer is coated with polyimide varnish followed by baking to form a polyimide support substrate 53 having a thickness of 2  $\mu\text{m}$ . (b) Then, a synthetic rubber type adhesive is applied onto the polyimide substrate, and is dried, and the polyimide substrate is immersed in an etching solution whose major components are chromic acid and sulfuric acid thereby roughening the surface of the adhesive layer 56 to improve the adhesion. (c) The surface of the adhesive layer 56 is activated by an acidic activating solution whose major components are palladium chloride and tin (II) chloride. Thereafter, a photoresist 57 is applied by the usual photo-process followed by baking to form a prescribed pattern, and development is effected to form a prescribed X-ray absorption pattern. (d) Then, a nickel underlay film 55 is deposited on the X-ray absorption pattern section where the activated adhesive layer surface is exposed by using an electroless nickel plating solution containing, as a major component, nickel sulfate, and as a reducing agent, sodium hypophosphite so that the nickel underlay film 55 may have a thickness of about 0.5  $\mu\text{m}$ . (e) By using a displacement gold plating solution whose major component is sodium dicyanoaurate (I), a displacement reaction between nickel and gold is allowed to take place so that a gold film 58 having a thickness of about 0.1  $\mu\text{m}$  may be deposited on the nickel underlay film. Thereafter, by using the above present electroless gold plating solution, gold 58 serving as a catalyst so that the gold 54 may have a thickness of about 0.6  $\mu\text{m}$ . (f) The silicon board 52 is formed with a hole 59 by using an etching solution whose major component is sodium hydroxide with the

undersurface of the silicon board formed with an etching mask. Finally, the photoresist, and the etching mask are removed.

As described above, according to the invention, the circumference effect (the phenomenon that an electric current is more concentrated to the circumferential section of an object to be plated than to the central part of the object and the thickness of plating at the circumferential section becomes greater than the central section) of the thickness of plating due to the electrical potential distribution which is a fundamental theme in electroplating did not occur, and therefore, an X-ray absorption pattern wherein the thickness of the coating is  $0.6 \pm 0.05 \mu\text{m}$  that is quite uniform could be formed. Thus, blur of the pattern at the circumferential section of the mask by the slant incident light of an X-ray could be reduced substantially.

Further, since in the present invention an underlay film for electricity supply that is essential in electroplating is not required, a step of etching an underlay film for masking the X-ray absorption pattern is not required, so that there were no possibilities that the lowering of the adhesion of the X-ray absorption pattern due to side etching would occur, and an X-ray absorption pattern having a size of 1  $\mu\text{m}$  or less and high in adhesion could be produced in a high yield.

Since in the present electroless gold plating solution, the solution temperature is 80° C., and the pH is 9, which are quite milder in comparison with those of the known cyanide type electroless gold plating solution that has a solution temperature of 90° C., and a pH of 13, a photoresist pattern need not be deformed. Further, since hydrogen gas is not released along with the deposition reaction of gold as in the case of a cyanide type electroless gold plating, release of a photoresist due to the release of hydrogen gas would not occur. Therefore, the formation of an X-ray pattern quite good in dimensional accuracy has become possible.

What is claimed is:

1. A method of plating with gold comprising the steps of:

immersing a substrate in an electroless gold plating solution comprising monovalent gold ions, said monovalent gold ions being supplied by reaction between a tetrahalogenoaurate (III) and a thiosulfate, a reducing agent, and a complexing agent which has a greater bond energy to a monovalent gold ion than a hydroxide ion has, said substrate having predetermined portions on which the gold is to be deposited; and

depositing gold on said predetermined portions of the substrate while said substrate is immersed in said electroless gold plating solution so as to form a gold layer on the predetermined portions of the substrate by electroless deposition, with substantially no deposition of gold on other portions of the substrate.

2. A method of plating with gold according to claim 1, characterized in that said tetrahalogenoaurate (III) is sodium tetrachloraurate (III), and said thiosulfate is sodium thiosulfate.

3. A method of plating with gold comprising the steps of:

immersing a substrate in an electroless gold plating solution comprising monovalent gold ions, thiourea as a reducing agent, and a complexing agent which has a greater bond energy to a monovalent gold ion than a hydroxide ion has, wherein said

monovalent gold ions and said complexing agent are supplied by the reaction between a tetrahalogenoaurate (III) and a thiosulfate, said substrate having predetermined portions on which gold is to be deposited; and  
 5  
 depositing gold on said predetermined portions of the substrate while said substrate is immersed in said electroless gold plating solution so as to form a gold layer on the predetermined portions of the substrate by electroless deposition, with substantially no deposition of gold on other portions of the substrate.

4. A method of plating with gold according to claim 3, characterized in that the content of said tetrahalogenoaurate (III) is 0.001 to 0.2 mol/l, the content of said thiosulfate is 0.001 to 0.9 mol/l, and the content of said thiourea is 0.001 to 1.0 mol/l.

5. A method of plating with gold according to claim 3, characterized in that the content of said tetrahalogenoaurate (III) is 0.006 to 0.05 mol/l, the content of said thiosulfate is 0.03 to 0.6 mol/l, and the content of said thiourea is 0.01 to 0.5 mol/l.

6. A method of plating with gold according to claim 3, characterized in that the content of said tetrahalogenoaurate (III) is 0.01 to 0.03 mol/l, the content of said thiosulfate is 0.04 to 0.2 mol/l, and the content of said thiourea is 0.02 to 0.3 mol/l.

7. A method of plating with gold comprising the steps of:

immersing a substrate in an electroless gold plating solution comprising monovalent gold ions, a reducing agent, and a complexing agent which has a greater bond energy to a monovalent gold ion than a hydroxide ion has, said substrate having predetermined portions on which gold is to be deposited, said electroless gold plating solution also containing a stabilizer, which is a sulfite, and a pH adjuster; and  
 30

depositing gold on said predetermined portions of the substrate while said substrate is immersed in said electroless gold plating solution so as to form a gold layer on the predetermined portions of the substrate by electroless deposition, with substantially no deposition of gold on other portions of the substrate.

8. A method of plating with gold according to claim 7, characterized in that the content of said sulfite is 0.01 to 0.8 mol/l, the content of said pH adjuster is 0.09 to 1.0 mol/l, the solution temperature is 60° to 90° C., and the pH of the plating solution is 7.0 to 11.0.

9. A method of plating with gold according to claim 7, characterized in that the content of said sulfite is 0.08 to 0.7 mol/l, the content of said pH adjuster is 0.4 to 1.0 mol/l, the solution temperature is 65 to 85° C., and the pH of the plating solution is 7.5 to 10.0.

10. A method of plating with gold according to claim 7, characterized in that the content of said sulfite is 0.15 to 0.6 mol/l, the content of said pH adjuster is 0.4 to 0.8 mol/l, the solution temperature is 70° to 80° C., and the pH of the plating solution is 8.0 to 9.0.

11. A method of plating with gold comprising the steps of:

immersing a substrate in an electroless gold plating solution comprising monovalent gold ions, a reducing agent consisting of thiourea, a complexing agent which has a greater bond energy to a monovalent gold ion than a hydroxide ion has, a pH regulator, and a stabilizer, wherein said gold ions

are supplied from a thiosulfate gold (I) complex whose content is 0.001 to 0.2 mol/l, and said complexing agent is a thiosulfate whose content is 0.001 to 0.05 mol/l, and wherein the content of thiourea is from 0.001 to 1.0 mol/l, said pH regulator is borax, said stabilizer is sodium sulfite, and the content of water is such as to make the total amount of said solution to 1 l, said substrate having predetermined portions on which gold is to be deposited; and  
 5

depositing gold on said predetermined portions of the substrate while said substrate is immersed in said electroless gold plating solution so as to form a gold layer on the predetermined portions of the substrate by electroless deposition, with substantially no deposition of gold on other portions of the substrate.

12. A method of plating with gold according to claim 11, wherein the content of borax is from 0.09 to 1.0 mol/l, and the content of sodium sulfite is from 0.01 to 0.8 mol/l.

13. A method of plating with gold comprising the steps of:

immersing a substrate in an electroless gold plating solution comprising monovalent gold ions, a reducing agent consisting of thiourea, a complexing agent which has a greater bond energy to a monovalent gold ion than a hydroxide ion has, a pH regulator, and a stabilizer, wherein said gold ions are supplied from a thiosulfate gold (I) complex whose content is 0.001 to 0.2 mol/l and said complexing agent is thiosulfate whose content is 0.001 to 0.5 mol/l, and wherein said thiosulfate gold (I) complex is a reaction product of a halogenoaurate (III) with a thiosulfate, said substrate having predetermined portions on which gold is to be deposited; and  
 20

depositing gold on said predetermined portions of the substrate while said substrate is immersed in said electroless gold plating solution so as to form a gold layer on the predetermined portions of the substrate by electroless deposition, with substantially no deposition of gold on other portions of the substrate.

14. A method of plating with gold comprising the steps of:

immersing a substrate in an electroless gold plating solution comprising monovalent gold ions, a reducing agent consisting of thiourea, a complexing agent which has a greater bond energy to a monovalent gold ion than a hydroxide ion has, a pH regulator, and a stabilizer, wherein the gold ions are supplied from a thiosulfate gold (I) complex whose content is 0.001 to 0.2 mol/l, and said complexing agent is a thiosulfate whose content is 0.001 to 0.5 mol/l, and wherein the thiosulfate gold (I) complex is a dithiosulfatoaurate (I), said substrate having predetermined portions on which gold is to be deposited; and  
 45

depositing gold on said predetermined portions of the substrate while said substrate is immersed in said electroless gold plating solution so as to form a gold layer on the predetermined portions of the substrate by electroless deposition, with substantially no deposition of gold on other portions of the substrate.